

# United States Patent

[111] 3,590,999

[72] Inventors Wayne D. Gould  
Miami, Ariz.;  
Guy H. Harris, Concord, Calif.  
[21] Appl. No. 799,119  
[22] Filed Feb. 13, 1969  
[45] Patented July 6, 1971  
[73] Assignee The Dow Chemical Company  
Midland, Mich.

[54] FLOTATION OF SULFIDE ORES  
10 Claims, No Drawings

[52] U.S. Cl. 209/166,  
260/455  
[51] Int. Cl. B03d 1/02  
[50] Field of Search. 209/166,  
167; 252/61; 260/455

[56] References Cited

UNITED STATES PATENTS

|           |         |          |           |
|-----------|---------|----------|-----------|
| 1,674,166 | 6/1928  | Douglass | 209/166   |
| 2,691,635 | 10/1954 | Harris   | 209/166 X |
| 3,118,924 | 1/1964  | Harman   | 260/455   |

FOREIGN PATENTS

187,116 12/1955 Austria 260/455

Primary Examiner—Frank W. Lutter

Assistant Examiner—Robert Halper

Attorneys—Griswold and Burdick, Bruce M. Kanuch and  
William R. Norris

**ABSTRACT:** An improvement in the concentration of ores by flotation which comprises subjecting a sulfide ore in the form of a pulp to a flotation process in the presence of an effective quantity of a flotation collector comprising a thiocarbamate compound corresponding to the formula



wherein X comprises a chelating group and R is hydrogen or a hydrocarbon radical containing from 1 to 10 carbon atoms; R<sub>1</sub> is an alkylene group, and R<sub>2</sub> is a hydrocarbon radical usually containing from 1 to 7 carbon atoms. Certain of the indicated compounds provide enhanced selectivity and/or recovery of sulfide minerals of Cu, Zn, Mo, Co, Ni, Pb and As over iron sulfide.

## FLOTATION OF SULFIDE ORES

## BACKGROUND

Flotation is a process of treating a mixture of finely divided mineral solids, e.g., a pulverulent ore, suspended in a liquid whereby a portion of such solids are separated from other finely divided mineral solids, e.g. clays and the like materials present in the ore, by introducing a gas (or providing a gas in situ) into the liquid to produce a frothy mass containing certain of the solids on the top of the liquid, and leaving suspended (unfrothed) other solid components of the ore. 10

Flotation is based on the principle that introducing a gas into a liquid containing solid particles of different materials suspended therein causes adherence of some gas to certain suspended solids and not to others and makes the particles having the gas thus adhered thereto lighter than the liquid. Accordingly, they rise to the top of the liquid to form a froth. 15

Various flotation agents have been admixed with the suspension to improve the frothing process. Such added agents are classed according to the function to be performed: collectors, e.g., high carbon chain compounds such as collectors for sulfide minerals including xanthates, thionocarbonates, and the like; frothers which impart the property of forming a stable froth, e.g., natural oils such as pine oil and eucalyptus oil; modifiers such as activators to induce flotation in the presence of a collector, e.g., copper sulfate; depressants, e.g., sodium cyanide, which tend to prevent a collector from functioning as such on a mineral which it is desired to retain in the liquid, and thereby discourage a substance from being carried up and forming a part of the froth; pH regulators to produce optimum metallurgical results, e.g., lime, soda ash and the like. 20

It is of importance to bear in mind that additaments of the above types are selected for use according to the nature of the ore, the mineral sought to be recovered, and the other additaments which are to be used in combination therewith.

An understanding of the phenomena which makes flotation a particularly valuable industrial operation is not essential to the practice of the present invention. They appear, however, to be largely associated with selective affinity of the surface of particulated solids, suspended in a liquid containing entrapped gas, for the liquid on one hand and the gas on the other.

The flotation principle is applied in a number of mineral separation processes among which is the selective separation of such minerals as sulfide copper minerals, sulfide zinc minerals, sulfide molybdenum minerals and others from sulfide iron minerals. The present invention concerns the use of an unique class of compounds as collection agents in a flotation process. With some of these collectors, better recoveries are realized and with others improved selectivity is achieved. Certain of these agents produce improvement in both aspects. 35

## SUMMARY

The present invention concerns an improved method of flotation separation of sulfide minerals which comprises subjecting a sulfide ore to a flotation process in the presence of a compound corresponding to the formula



wherein R represents H, or a hydrocarbyl radical containing from 1 to 10 carbons, R<sub>1</sub> is a divalent hydrocarbon moiety containing from 1 to 7 carbons, R<sub>2</sub> is a hydrocarbyl radical containing from 1 to 7 carbons and X is a chelating group.

These compounds are useful as flotation collectors in flotation processes for the concentration of sulfide minerals such as copper, zinc, molybdenum, cobalt, nickel, lead and arsenic from ores in preference to other minerals. 75

## PREFERRED EMBODIMENTS

In the practice of the present invention, the defined class of compounds are employed as flotation collectors using standard flotation technique. Preferably, the compounds employed correspond to the formula



wherein X corresponds to a chelating group selected from the group consisting of



R corresponds to H (when X is other than



), or a hydrocarbyl radical selected from the group consisting of an alkyl or alkenyl group, preferably containing from 1 to 10 carbon atoms, an aryl, cycloalkyl, aralkyl, alkaryl or an aralkenyl group; R<sub>1</sub> corresponds to an alkylene group, preferably containing from 1 to 5 carbon atoms, and R<sub>2</sub> corresponds to a hydrocarbyl radical selected from the group consisting of an alkyl or an alkenyl group preferably containing from 1 to 7 carbon atoms, a cycloalkyl, cycloalkenyl, aralkyl, or aralkenyl group. Preferably R represents H when R<sub>1</sub> contains 3 or more carbon atoms and X is other than



It appears that the presence of the chelating group in the flotation collector compound as defined herein allows for better and more selective flotation of certain sulfide minerals over the use of otherwise similar thiocarbamate flotation collectors heretofore employed. 40

The flotation collector compounds as defined herein are particularly effective in flotation processes used to separate and concentrate copper sulfide and similar minerals from sulfide ores. In such process, a pulp is first prepared by wet grinding a sulfide containing ore to a suitable particle size, with or without a pH modifier. A suitable frothing agent is then added, e.g., pine oil, cresylic acid, polyalkoxyparaffin and the like. An effective quantity of the flotation collector compound, as defined herein, is then added in an amount usually ranging from about 0.01 lb. to about 0.25 lb. per ton of pulp and the pulp is then agitated and aerated. The copper sulfide minerals and other like sulfide minerals collect as a froth which is readily overflowed or skimmed off from the residual gangue and nondesired materials and the metal values therein recovered. 45

The following Examples will facilitate a more complete understanding of the present invention but they are not meant to limit the scope of the invention to the specific embodiments 50 incorporated therein.

## EXAMPLE 1

Various species of flotation collector compounds within the scope of the present invention were employed in the flotation recovery of copper values from a sulfide ore obtained from South America employing the following procedure: An ore sample was wet ground for 5 minutes at 66 percent by weight solids with no other reagents. The pulp was then conditioned 55 for 8 minutes by mixing with 0.12 lb./ton of a flotation collector to be evaluated and 0.13 lb./ton of a standard frother. During the conditioning period, the pH was adjusted by the addition of a mineral acid to a value of about 3.8. The pulp was then floated by aeration for 7 minutes and the tailings assayed 60 for copper.

Employed as a control for comparison purposes was a standard flotation collector compound consisting of a thiocarbamate compound corresponding to the formula:



The specific collector compounds of the present invention employed, and recoveries are set forth in the following Table I

TABLE I

It will be observed that the flotation collectors of the invention performed as well as, or better than, the control collector.

### EXAMPLE 2

Some of the collectors employed in Example 1 were further tested on a copper sulfide ore obtained from the Southwestern United States. The ore sample was ground for 4  $\frac{1}{2}$  minutes at 59 percent solids with 2.0 lbs./ton of lime. The pulp was conditioned for 2 minutes with an amount of a specific collector and

0.16 lb./ton of a standard frother at a pH of 10.5. The pulp was then floated 8 ½ minutes and the tailings assayed for copper. The collector composition and results obtained are set forth in the following Table II. The same control flotation collector was employed as in Example 1.

### EXAMPLE 3

In this example, copper sulfide and molybdenum sulfide containing ores were treated in a manner similar to that described in the foregoing examples. Used as controls were the prior art flotation collector employed in Example 1 (Con-



trol 1) and a second collector (Control 2) corresponding to the formula:

75 Comparatively evaluated was the new flotation collector com-

TABLE II

| Run No.      | Collector Compound                                                                                      | Lb./ton added | Percent Cu in tail | Percent Cu recovery |
|--------------|---------------------------------------------------------------------------------------------------------|---------------|--------------------|---------------------|
| Control..... | Control.....                                                                                            | .0025         | 0.330              | 59.6                |
| 1.....       | $\text{H}_3\text{COCH}_2\text{CH}_2\text{N}(\text{HS})\text{COCH}_2(\text{CH}_3)_2$                     | .0025         | 0.305              | 63.6                |
| 2.....       | $\text{H}_3\text{CSCH}_2\text{CH}_2\text{N}(\text{HS})\text{COCH}(\text{CH}_3)_2$                       | .0025         | 0.261              | 68.1                |
| Control..... | Control.....                                                                                            | .0125         | 0.288              | 66.1                |
| 3.....       | $\text{H}_3\text{COCH}_2\text{CH}_2\text{CH}_2\text{N}(\text{HS})\text{COCH}_2\text{CH}(\text{CH}_3)_2$ | .0125         | 0.240              | 71.0                |
| 4.....       | $\text{H}_3\text{CSCH}_2\text{CH}_2\text{N}(\text{HS})\text{COCH}_2\text{CH}_2\text{CH}(\text{CH}_3)_2$ | .0125         | 0.215              | 74.2                |
| 5.....       | $\text{H}_{17}\text{C}_8\text{SCH}_2\text{CH}_2\text{N}(\text{HS})\text{COCH}_2\text{CH}_3$             | .0125         | 0.259              | 68.6                |
| 6.....       | $\text{H}_3\text{CSCH}_2\text{CH}_2\text{CH}_2\text{N}(\text{HS})\text{COCH}(\text{CH}_3)_2$            | .0125         | 0.239              | 71.2                |
| 7.....       | $\text{HSCH}_2\text{CH}_2\text{N}(\text{HS})\text{COCH}(\text{CH}_3)_2$                                 | .0125         | 0.268              | 67.5                |
| 8.....       | $\phi\text{SCH}_2\text{CH}_2\text{N}(\text{HS})\text{COCH}(\text{CH}_3)_2^a$                            | .0125         | 0.235              | 71.6                |
| 9.....       | $\phi\text{CH}_2\text{SCH}_2\text{CH}_2\text{N}(\text{HS})\text{COCH}(\text{CH}_3)_2$                   | .0125         | 0.240              | 71.1                |

pound having the formula:



The process conditions and results of this study are tabulated in following Table III.



wherein  $R_2$  is the same as defined hereinbefore, and  $M^+$  is an alkali metal cation, with an amine containing a chelating group in the carbon chain corresponding to the general formula

TABLE III

| Ore source       | Collector                                                                                          | Amount of collector, lb./ton pulp | Standard frother, lb./ton | Diesel oil, lb./ton | pH  | Conc. of minerals in feed stock, percent |       | Recovery, percent |       | Tails, percent |        |
|------------------|----------------------------------------------------------------------------------------------------|-----------------------------------|---------------------------|---------------------|-----|------------------------------------------|-------|-------------------|-------|----------------|--------|
|                  |                                                                                                    |                                   |                           |                     |     | Cu                                       | Mo    | Cu                | Mo    | Cu             | Mo     |
| South America    | Control (1)                                                                                        | 0.06                              | 0.134                     | 0.033               | 4.5 | 19.27                                    | 0.330 | 84.66             | 61.78 | 0.281          | 0.0164 |
| Do.              | $\text{H}_3\text{COCH}_2\text{CH}_2\text{CH}_2\text{NC(OCH}_2\text{CH}_2\text{COH(CH}_3\text{)}_2$ | 0.06                              | 0.134                     | 0.033               | 4.5 | 19.76                                    | 0.326 | 89.00             | 62.59 | 0.202          | 0.0164 |
| Southwest U.S.A. | Control (2)                                                                                        | 0.01                              | 0.100                     | 0.00                | 8.5 | 11.93                                    | 0.395 | 68.16             | 85.48 | 0.265          | 0.0032 |
| Do.              | $\text{H}_3\text{COCH}_2\text{CH}_2\text{CH}_2\text{NC(OCH}_2\text{CH}_2\text{COH(CH}_3\text{)}_2$ | 0.01                              | 0.110                     | 0.00                | 8.5 | 15.20                                    | 0.469 | 74.23             | 86.71 | 0.213          | 0.0029 |

**EXAMPLE 4**

**EXAMPLE 4**  
A zinc sulfide containing ore was treated as in the foregoing examples employing the same control collector as in Example 1 and a collector compound within the scope of the present invention corresponding to the formula:



The process conditions and results of this study are tabulated in the following Table IV.

la R-X-R<sub>1</sub>-NH<sub>2</sub> wherein R, X and R<sub>1</sub>, are the same as defined hereinbefore.

Other collector compounds are prepared by reacting an isothiocyanate compound, containing a chelating group, corresponding to the general formula  $R-X-R_1-N=C=S$  wherein R, X and R<sub>1</sub> are the same as defined hereinbefore; with an alcohol corresponding to the general formula  $R_2OH$  wherein R<sub>2</sub> is the same as defined hereinbefore.

Still other collectors of the invention are obtained by multistage preparative reactions. For example, when a thiol

TABLE IV

| Ore source     | Collector     | Amount of collector, lb./ton | Standard frother, lb./ton | Pine oil, lb./ton | CuSO <sub>4</sub> , lb./ton | Conc., percent Zn | Recovery, percent Zn | Tails, percent Zn |
|----------------|---------------|------------------------------|---------------------------|-------------------|-----------------------------|-------------------|----------------------|-------------------|
| Eastern Canada | Control       | 0.039                        | 0.028                     | 0.045             | 0.39                        | 14.87             | 58.1                 | 1.15              |
| Do.            | New collector | 0.033                        | 0.024                     | 0.043             | 0.55                        | 20.57             | 80.0                 | 0.41              |

Flotation collectors as defined herein are prepared by several methods well known in the art. For example, the compounds are prepared by the reaction of a xanthate compound corresponding to the general formula

compound corresponding to the formula  $RSH$ , wherein  $R$  is the same as hereinbefore defined, is contacted with ethylenimine, as amine compound corresponding to the formula  $R-S-CH_2CH_2NH_2$  is formed. This product is then con-

tacted with a xanthate ester to prepare a compound within the scope of the present invention corresponding to the formula



wherein  $\text{R}_2$  is the same as defined hereinbefore. Other amine compound starting materials can be prepared by methods well known in the art. For example, reference may be made to Wagner & Zook, *Synthetic Organic Chemistry* PP 787-796, 801-805 (1953).

In another preparative process a compound corresponding to the formula



Y

wherein Y is H or a lower alkyl, is reacted with an alcohol or thiol compound corresponding to the formulas  $\text{ROH}$ ,  $\text{RSH}$  respectively, wherein R is the same as defined hereinbefore, to prepare compounds corresponding to the formulas  $\text{ROCH}_2\text{CHY-N}$ ,  $\text{RSCH}_2\text{CHY-CN}$ , respectively. These compounds are then contacted with a reducing agent such as  $\text{LiAlH}_4$  or  $\text{H}_2$  over a catalyst to provide compounds corresponding to the formulas



and



respectively. These products are then reacted with a xanthate ester to provide products corresponding to the formulas



and



respectively, wherein  $\text{R}_2$  is the same as previously defined.

The xanthates starting materials can be prepared by reacting a solution of an alkali metal hydroxide or alkoxide in an alcohol corresponding to the formula  $\text{R}_2\text{OH}$ , wherein  $\text{R}_2$  is the same as defined hereinbefore, with carbon disulfide ( $\text{CS}_2$ ) and then with methyl chloride to provide a xanthate compound corresponding to the formula



wherein  $\text{R}_2$  is the same as defined hereinbefore. Other starting materials and process schemes can also be employed in preparing the flotation collectors useful in the process of the present invention.

One species of a flotation collector for use in the process of the scope of the present invention, corresponding to the formula



was prepared by adding 19.2 grams of technical grade methyl isopropylxanthate to 15.2 grams of a compound corresponding to the formula



at room temperature. The ensuing exothermic reaction was allowed to proceed to substantial completion as evidenced by a subsidence of the temperature of the reaction mixture. The product, an oil, was heated on a steam bath and an inert gas was passed through it to remove any residual mercaptan. Elemental analysis of the product showed 6.33 weight percent sulfur. Calculated analysis for sulfur in the compound corresponding to the formula set forth herein is 6.2 percent.

Another collector of the invention corresponding to the formula



was prepared as follows: Sodium methyl mercaptide was

reacted with 4-bromobutyronitrile to give a compound which, when reduced with  $\text{LiAlH}_4$ , gave an amine starting material corresponding to the formula  $\text{CH}_3-\text{S}-(\text{CH}_2)_4\text{NH}_2$ . To 10.5 grams of methyl isopropylxanthate was added 8.3 grams of the amine starting material. After the spontaneous evolution of  $\text{CH}_3\text{SH}$  had subsided, the reaction mixture was heated on a steam bath for about 3 hours. At the end of this period, the remaining  $\text{CH}_3\text{SH}$  was removed by heating the reaction mixture to  $70^\circ\text{C}$ . under a 20 mm. reduced pressure and the resulting product separated.

This compound is useful as a flotation collector in the flotation separation of sulfide mineral containing ores.

Another collector compound corresponding to the formula



was prepared as follows: To 250 ml. of alcohol was added 3 grams of  $\text{NaOH}$  and to the resulting solution was added 13 grams (0.075 moles) of



To this mixture was added 10.2 grams (0.068 mole) of methyl ethylxanthate, and the resulting mixture refluxed until the evolution of  $\text{CH}_3\text{SH}$  ceased. The excess base was neutralized with  $\text{CO}_2$  and the reaction mixture was evaporated to dryness. The resulting residue was extracted with chloroform, filtered, and the filtrate evaporated to dryness. The product was recrystallized from isopropanol. The product yield was 12.5 grams of a solid which had a melting point range of about  $70.5-71.5^\circ\text{C}$ . This compound is also useful as a flotation collector in sulfide mineral flotation processes.

In a manner similar to that described directly above, 3-methylsulfenyl propyl amine is reacted with methyl ethylxanthate to provide a compound corresponding to the formula



This compound can also be employed as a flotation collector in typical mineral sulfide flotation processes.

Examples of other alcohols which can be employed in the above preparations of the collector compounds include, cyclohexanol, cyclohexenol, allyl alcohol, cinnamyl alcohol, crotyl alcohol; 2, 3, 5-trimethyl-3-hexanol and 2,3,4-trimethyl-2-hexanol.

Examples of amine compounds which can be employed in the preparation of collector compounds include



Xanthate compounds which can be employed in place of those described above to prepare collector compounds of the invention herein, by other methods known in the art include, for example



and the like.

Other compounds useful as flotation collectors, are prepared in a manner similar to those set forth hereinbefore and are characterized by the general formula



wherein R, X,  $\text{R}_1$  and  $\text{R}_2$  are as set forth in the following Table V.

TABLE V

| R                                                                                   | X                                                   | R                                                                                 | R <sub>2</sub>                                                                    |
|-------------------------------------------------------------------------------------|-----------------------------------------------------|-----------------------------------------------------------------------------------|-----------------------------------------------------------------------------------|
|    | SO                                                  |  |  |
|    | SO                                                  |  |  |
|    |                                                     |                                                                                   |  |
|    | SO                                                  |  |  |
|    |                                                     |                                                                                   |                                                                                   |
|    | SO                                                  |  |  |
|    | CH <sub>3</sub> -CH <sub>2</sub> -CH <sub>2</sub> - | -S-                                                                               |  |
|    |                                                     |                                                                                   |                                                                                   |
| H-                                                                                  |                                                     | -O-                                                                               |  |
| C <sub>3</sub> H <sub>7</sub> -                                                     | SO <sub>2</sub>                                     |  |  |
| C <sub>2</sub> H <sub>5</sub> -                                                     |                                                     |                                                                                   |                                                                                   |
|    |                                                     |                                                                                   |                                                                                   |
| H-                                                                                  |                                                     | -O-                                                                               |  |
| C <sub>3</sub> H <sub>7</sub> -                                                     |                                                     |                                                                                   |                                                                                   |
|    |                                                     |                                                                                   |                                                                                   |
|  |                                                     |                                                                                   |                                                                                   |
| H-                                                                                  |                                                     |                                                                                   |                                                                                   |
|  |                                                     |                                                                                   |                                                                                   |

Various modifications may be made in the present invention without departing from the spirit or scope thereof for it is understood that we are limited only as defined in the appended claims.

We claim:

1. In the process of concentrating sulfide ores by froth flotation in the presence of a flotation collector the improvement which comprises:



wherein R represents a member selected from the group consisting of H, an alkyl, alkenyl, aryl, aralkyl, aralkenyl, cycloalkyl, alkaryl or a cycloalkenyl group; R<sub>1</sub> is an alkylene group containing from 1 to 5 carbon atoms; R<sub>2</sub> is a hydrocarbyl radical selected from the group consisting of alkyl, alkenyl, cycloalkyl, cycloalkenyl, aralkyl or an aralkenyl group and "X" represents a chelating member selected from the group consisting of

—O—, —S—, SO and SO<sub>2</sub>

and the compound is further characterized in that when X is a member selected from the group consisting of SO or SO<sub>2</sub>, R is not H.

2. The process as defined in claim 1 wherein R represents a member selected from the group consisting of H, an alkyl or alkenyl group containing from 1 to 10 carbon atoms, R<sub>1</sub> is a

member selected from the group consisting of alkyl or alkenyl groups containing from 1 to 7 carbon atoms and X represents a chelating member selected from the group consisting of

50

—O—, —S—,  $\overset{\cdot}{S}O$  and  $\overset{\cdot}{S}O_2$

and the compound is further characterized in that when X is a member selected from the group consisting of

S O or S O<sub>2</sub>,

R is not H.

3. The process as defined in claim 1 wherein from about 0.01 to about 0.25 pound of said collector is employed per ton of ore pulp treated.

4. The process as defined in claim 1 wherein the flotation collector is a compound corresponding to the formula

$$\text{CH}_3\text{SCH}_2\text{CH}_2\text{NCOCH}(\text{CH}_3)_2$$

5. The process as defined in claim 1 wherein the flotation collector is a compound corresponding to the formula

70 
$$\text{H} \quad \text{S}$$
  

$$(\text{CH}_2)_5\text{CH}=\text{CH}_2 \text{CH}_2\text{N}=\text{OCH}(\text{CH}_3)_2$$

6. The process as defined in claim 1 wherein the flotation collector is a compound corresponding to the formula

7. The process as defined in claim 1, wherein the substituent

collector is a compound corresponding to the formula

H S



8. The process as defined in claim 1 wherein the flotation 5  
collector is a compound corresponding to the formula



H S



9. The process as defined in claim 1 wherein the flotation

collector is a compound corresponding to the formula



H S



10. The process as defined in claim 1 wherein the flotation  
collector is a compound corresponding to the formula

10



15

20

25

30

35

40

45

50

55

60

65

70

75